

C. W. Stafford,  
Casting Car Wheels.

No 44,120.

Patented Sep. 6, 1864.



Witnesses;  
W. J. Demis  
Charles D. Smith

Inventor;  
W. Stafford

# UNITED STATES PATENT OFFICE.

CHARLES W. STAFFORD, OF SAYBROOK, CONNECTICUT.

## IMPROVED CAST-STEEL CAR-WHEEL.

Specification forming part of Letters Patent No. 44,120, dated September 6, 1864.

*To all whom it may concern:*

Be it known that I, CHARLES W. STAFFORD, of Saybrook, Connecticut, have invented a new and useful Mode or Process of Casting Cast-Steel Car-Wheels; and I do hereby declare that the following is a full and exact description thereof, reference being had to the accompanying drawings, and to the letters of reference marked thereon.

The nature of my invention consists in the use of a cast-iron or other suitable metallic shell or core of proper shape for the interior surface of the car-wheel, said shell or core being rigidly supported within a cast-iron or other suitable flask or mold made of the desired form of the exterior surface of the wheel, said flask or mold being provided with proper pouring-gates, through which the molten steel is poured, directly from the crucible or otherwise, upon and around the shell or core, and being thereby thoroughly amalgamated and welded thereto, thus forming a perfect and solid wheel, the inside surface of which is of cast-iron or other suitable metal, and the outer or wearing surface is of cast-steel.

To prevent the shell or core from becoming too much heated by the molten steel while pouring, I make the core or shell hollow, and fill the cavity thereof with sand or other suitable material, and perforate the same with air-passages for conveying off the gases and surplus heat.

In the drawings which accompany this specification and form a part thereof, Figure 1 represents a top view of the metallic flask with one-half the top removed. Fig. 2 represents a cross-section of the flask and core. Fig. 3 represents a cross-section of the same at the red line *o o*.

To enable those skilled in the art to construct and use my invention, I will now proceed to describe the same.

A, Fig. 1, is a metallic mold or flask, the top of which, A', may be constructed in one or more parts, and which is provided with one or more pouring-gates, *c c*. The flask is also provided with bolts or standards 5 5 5 5,

which are fitted with keys 6 6 6 6, for holding the sections of the flask together and secure the same when ready for use. The flask may be further provided with holes or openings, as desired, for the escape of air and to prevent "blowing" in the process of pouring.

I construct the iron core or shell 2 2, Figs. 2 and 3, which composes the inner surface of the hollow body of the wheel, in any of the ordinary forms. The numerals 1 1, Figs. 2 and 3, represent the cavity between the outer surface of the core 2 2 and the inside surface of the flask A B, and corresponds with the outside of the wheel when cast. The core is made hollow, and its cavity 3 3, Fig. 2, is filled with sand or other suitable material.

B represents the lower section of the flask A, and through a hole in its center passes a bolt or standard, *d*, secured to the bottom of the flask B by the nut *e*, and, while passing through the core 2, securing the same in its proper position, and fitting snugly at its upper end in the center of the top of the flask A'. The top of the flask A' is further provided with one or more pouring-gates, *c c*, through which the melted metal reaches the cavity, and filling the space 1 1 forms the wheel. In the sand which fills the cavity of the core 2, I make perforations, as may be seen at 4 4, to give vent to the gases or surplus heat generated during the process of pouring.

What I claim as my invention, and desire to secure by Letters Patent, is—

1. The employment, in the casting of cast-steel car-wheels or other cast-steel castings, of a shell or core made of metal filled with sand, together with the bolt *d*, or other similar device, in combination with a metallic flask or mold, as and for the purposes described.

2. As an article of manufacture, a cast-steel car-wheel, when the same is made as described.

C. W. STAFFORD.

Witnesses:

C. D. SMITH,  
W. F. DENNIS.